

Aug. 4, 1931.

L. W. MELCHER

1,817,388

METHOD AND APPARATUS FOR CASTING JOURNAL BOXES

Filed Feb. 16, 1929



Fig. 2



Inventor  
Lee W. Melcher  
By Fred Gerlach Atty.

## UNITED STATES PATENT OFFICE

LEE W. MELCHER, OF DE PERE, WISCONSIN, ASSIGNOR TO FAFNIR BEARING COMPANY, OF NEW BRITAIN, CONNECTICUT, A CORPORATION OF CONNECTICUT.

## METHOD AND APPARATUS FOR CASTING JOURNAL BOXES

Application filed February 16, 1929. Serial No. 340,477.

The invention relates to casting journal boxes for roller-bearings. In these boxes it is advantageous to form an integral cylindrical wall having a bearing surface for the rollers to avoid the necessity of a separate hard metal bearing sleeve. It is also advantageous to form the upper portion or load zone of the integral wall of hard metal in order to resist wear.

10 In journal boxes of the aforementioned character, it is necessary that the load zone of hard metal in the cylindrical wall should be of sufficient thickness to form a structure which will be reliably resistant to wear for 15 a long period of time, after it has been ground or finished. One object of the present invention is to provide an improved method of producing journal boxes in which the load zone of the cylindrical wall will be 20 hardened and of sufficient depth to withstand efficiently wear.

Another object of the invention is to provide an improved method of producing journal boxes of this character, in which the 25 impurities in the molten metal are kept away from that portion of the cylindrical wall in which the load zone is formed and are caused to accumulate in a portion of the box which is not used as a bearing surface.

30 A further object of the invention is to provide an improved method of casting journal boxes in which the sides and top of the journal box, as well as the pedestal guides and equalizer seats are formed of hard metal.

35 A still further object of the invention is to provide an improved mold for use in casting journal boxes having an integral cylindrical bearing wall.

40 Other objects of the invention will be apparent from a consideration of the following detailed description.

The invention consists in the several novel features hereinafter set forth and more particularly defined by claims at the conclusion 45 hereof.

In the drawings which accompany and form a part of this specification or disclosure and in which like numerals of reference denote corresponding parts throughout the several views; Fig. 1 is a section of a mould

showing the preferred manner of carrying out the invention. Fig. 2 is a section taken on the line 2-2 of Fig. 1. Fig. 3 is a section of the journal box produced by the present method and in the improved mould.

The invention is exemplified in assembling certain cores in a flask which comprises a cope 4 and a drag 5. The flask is first placed on a bottom-board 6. A bed 7 of sand is then packed on said board. A dry-sand core 8, which has its top face shaped to form the bottom  $a'$  of the journal box  $a$  is then placed upon the sandbed 7. Chill-sections 12, with dry-sand cores 13 baked on the outer sides thereof, are laid on the bottom-core 8. These sections 12 are shaped and spaced apart to cause a layer  $a''$  of hard metal at the side-faces  $a^3$  of the box  $a$ , and are provided with vertical grooves 14 in their inner faces, to form hard-metal pedestal guides  $a^5$  on the sides of the box. Dry-sand cores 9, which are shaped to form the end-walls of the box  $a$ , are placed on the bottom-core 8 and across the ends of the chill-sections 12 and cores 13.

A cylindrical opening  $a^6$  is formed in the box to provide an integral correspondingly cylindrical bearing-wall  $a^7$  or race in the box  $a$ , for a series of rollers around an axle in the box. This wall  $a^7$  is formed by a composite core which is held in prints in and extending 50 across the space between the end-cores 9. This composite core consists of a chill-section 18 and a dry-sand section 19 which are baked together and have their peripheral portions shaped to form the cylindrical opening  $a^6$  in the casting. The periphery 18 of chill-section 18 extends throughout less than 180°, preferably about 160°, of opening  $a^6$ , to form a hard-metal zone  $a^8$  of corresponding area 55 which constitutes the load zone of the bearing wall  $a^7$ . Dry-sand section 19 forms the remainder of the wall  $a^7$  of soft metal. The bottom face of chill-section 18 is recessed, and sand section 19 extends into the recess, so the two sections will remain corelatively 60 positioned to form truly the opening  $a^6$ . The composite core is positioned so the axis of opening  $a^6$  will be horizontal and the chill-section 18 is placed at the top, for the purpose hereinafter described. Dry-sand cores 65

20 are held in core-prints in end-cores 9 and extend longitudinally across the space around the chill-section 18 and core 19, to form holes 5  $a^{10}$  in the casting for bolts which extend through the box to secure the usual end cap and inner retaining ring thereon. Dry-sand cores 21 are supported in prints in end-cores 9, to form an oil-well in the bottom of the box. A dry-sand core 15<sup>a</sup>, with a chill-section 15 baked thereon, is placed on and 10 extends over the top of the end cores 9 and chill-sections 12 and cores 13. Section 15 forms a hard metal face  $a^{11}$  on the top of the box  $a$ , and has a recess 15<sup>b</sup> to form a hard-metal 15 equalizer seat  $a^o$  on the top of the box, and cross-grooves 15<sup>a</sup> to form hard metal guide- 20 ribs  $a^{12}$  for the equalizer bar, at the ends of seat  $a^o$ . After the parts of the mold have been assembled in the flask, the space 7<sup>a</sup> between the walls of the flask and the side-cores 13 and end-cores 9, is filled with sand so that the mold will be surrounded by sand to permit expansion of the parts of the mold. A vertical gate 23 extends downwardly 25 through top-core 15<sup>a</sup> and one of the side cores 13 to a horizontal gate 24 in bottom-core 8 below chill 12. The gate 24 is connected by a restricted upwardly extending gate 25 to the space which is to be filled with 30 metal. One or more gas vents (not shown) extend through the chill 15 and core 15<sup>a</sup>.

In practice it has been found that if the metal is permitted to boil or to be excessively agitated during the process of pouring, only 35 a comparatively thin film of metal will be hardened by the chill-sections so that the hardened zone will not be effective to prevent wear particularly on the cylindrical bearing surface. It has also been found that when the temperature of the various chill-sections is too low, the metal will boil or be agitated excessively and displace the previously deposited portions on the chill-section, and to minimize this, the chill-sections are heated 40 approximately to 180° Fahrenheit. The chills are heated to somewhat higher temperature before they are placed in the mold, and the period of pouring with respect to the closing of the moulds is timed to maintain 45 the temperature of approximately 180° Fahrenheit at the commencement of the pouring operation. All parts of the mould which form soft metal portions of the box are formed of dry-sand cores, to minimize the 50 agitation which results from the production of gas by moisture in the mould.

When the mould has been prepared as set forth, the molten metal, at approximately 55 2500° Fahrenheit is poured into the gate 23, from which it flows through the gate 24 and then upwardly through the restricted gate 25 into the bottom of the space in which the box is formed. In pouring, a constant supply of molten metal is maintained in the 60 down-gate by reason of the restriction in the

up-gate 25, so that the molten metal will flow into the mould with a uniform pressure to avoid surging and cold shuts in the chilled or other surfaces of the casting. The molten metal entering the mould from the bottom 70 will progressively fill up the space, and after the lower portion has been filled, it will rise between the sides of the core 19 and chill-section 12. The molten metal will flow approximately in the directions indicated by 75 the arrows, and, as it rises above the lower edge of the chill-section 18, it progressively flows over the peripheral face of the chill-section 18, and the subsequently incoming metal will rise adjacent the side chills without displacing the metal which has been 80 previously deposited on the periphery of chill-section 18. In practice it has been found that any flow of the molten metal over 85 previously deposited metal on a chill will have the effect of reducing the thickness of the hardened zone. As a result, the zone of metal hardened by the chill 18 will be of sufficient thickness, for example  $\frac{1}{8}$  of an inch, to form an effective hard metal bearing 90 surface in the load zone in, and integral with, the cylindrical bearing wall. The impurities in the metal, by reason of avoiding excessive agitation, will remain on the top of the flux and accumulate at the top of the 95 box and will not be deposited on the load zone of the cylindrical wall. This is important, because the presence of impurities in the load zone is objectionable, while their presence is not objectionable in 100 the top of the box which is not used as a bearing surface. During this pouring, the metal flows upwardly between the constricted portions of the spaces at the sides of the core 19 and the chill 12, and, as 105 a result, the zone of hard metal at the central side portions of the box may be somewhat irregular in depth or narrower than the hard metal in the load zone of the cylindrical wall. This however is of no moment, 110 because such portions of the box are not subjected to great wear. The pouring of the metal is continued until the entire space in the mould has been filled. Chill-section 15 forms a hard metal portion on which the 115 equalizer seat is formed so that it will resist wear. The chill-sections 12 harden the metal in the sides of the box and in the pedestal guides to render them wear-resisting. In cooling, the expansion of the metal will 120 contract the opening  $a^o$  and force the chill-section 18 downwardly and toward the center of the cylindrical wall and will crush the sand-core 19. This eliminates shrink cracks and distortion of the cylindrical wall of the 125 box which would otherwise result from the expansion of the metal and contraction of the cylindrical wall, and also facilitates the removal of the chill.

The invention exemplifies a method of 130

casting journal boxes with an integral cylindrical wall for a bearing surface with a hardened portion in the load zone of sufficient thickness to be effective and to permit the necessary finishing or grinding. It also exemplifies a casting method which produces a load zone of hard metal in the cylindrical wall of uniform thickness and comparatively free from defects caused by impurities in the metal. It also exemplifies an improved method by which uniform castings will be produced at a low cost.

The invention is not to be understood as restricted to the details set forth, since these may be modified within the scope of the appended claims, without departing from the spirit and scope of the invention.

Having thus described the invention, what I claim as new and desire to secure by Letters Patent, is:

1. The method of casting a journal box having an integral cylindrical bearing wall, which consists in preparing a mould with a chill section shaped to form a hard metal load zone in said cylindrical wall and arranged so that its periphery faces upwardly and extends horizontally, and with a core to form the remainder of the cylindrical wall, and pouring metal from below into the cavity around the core and chill section so it will flow upwardly and progressively over the periphery of the section to form the hardened load zone without displacing any substantial portion of the metal previously deposited on the chill-section.

2. The method of casting a journal box having an integral cylindrical bearing wall, which consists in preparing a mould with a chill-section shaped to form a hard metal load zone of less than 180° in said cylindrical wall, arranged so that its periphery faces upwardly and extends horizontally, and with a core to form the remainder of the cylindrical wall, and pouring metal from below into the cavity around the core and chill member so it will flow upwardly and progressively over the periphery of the section to form the load zone without displacing any substantial portion of the metal previously deposited on the chill-section and cause said zone to be comparatively thick.

3. The method of casting a journal box having an integral cylindrical bearing wall, which consists in preparing a mould with a chill-section adapted to form a hard metal load zone in said cylindrical wall and arranged so that its periphery faces upwardly and extends horizontally, and with a sand core to form the remainder of the cylindrical wall, pouring metal from below under uniform pressure and restricted flow into the cavity around the core and chill-section so it will flow upwardly and progressively over the periphery of the section and form the load zone without displacing any substan-

tial portion of the metal previously deposited on the chill-section so that it is comparatively thick.

4. The method of casting a journal box having an integral cylindrical bearing-wall, which consists in preparing a mould with a chill-section shaped to form a hard metal load zone of less than 180° of the cylindrical wall and arranged so that its periphery faces upwardly, and with a crushable sand core shaped to form the remainder of the cylindrical wall of soft metal and adapted to permit the chill-section to be forced toward the center of the opening by the expansion of the metal, and pouring metal from below into the space around the core and chill-section, so it will progressively flow over the periphery of the chill-section without displacement.

5. The method of casting a journal box having an internal cylindrical bearing wall, which consists in preparing a mould with chill-sections shaped to form the sides of the box, a chill-section shaped to form a zone of hard metal of less than 180° in the cylindrical wall with its periphery facing upwardly, a sand core to form the remainder of the cylindrical wall, and pouring metal from below into the cavity around the core and between the chill-sections.

6. The method of casting a journal box having an integral cylindrical bearing wall, which consists in preparing a mould with chill sections shaped to form the sides and top of the box, a cylindrical chill-section shaped to form a zone of hard metal of less than 180° in the cylindrical wall, a dry sand core to form the remainder of the cylindrical wall and a dry sand core to form the bottom of the box of soft metal, and pouring metal from below into the cavity around the first mentioned core and between the chill-sections.

7. The method of casting a journal box having an integral cylindrical bearing wall, which consists in preparing a mould with chill-sections to form the sides and top of the box, a cylindrical chill-section shaped to form a zone of hard metal in the cylindrical wall, and a dry-sand filling to form the bottom of the box of soft metal, and with cores to form bolt holes extending through the box, and pouring metal from below into the cavity around the core and between the chill-sections.

8. The method of casting a journal box having an integral cylindrical bearing wall, which consists in preparing a mould with chill sections to form the sides, a chill-section to form the top of the box having a recess therein to form an equalizer seat of hard metal, a chill section shaped to form a zone of hard metal in the cylindrical wall, a sand core to form the remainder of the cylindrical surface and a dry sand filling to form the bottom of the box of soft metal, and pouring

- metal from below into the cavity around the core and between the chill sections.
9. A mould for journal boxes having an integral cylindrical bearing wall, comprising a flask, a chill section positioned in the mould cavity and shaped to form an upper zone of hard metal in the cylindrical wall, and means forming a gate leading upwardly to the space below the core.
10. A mould for a journal box having an integral cylindrical bearing wall, comprising a flask, a chill section and a sand section united together to form a composite core and arranged with the chill-section on top and in the mold cavity so as to form the cylindrical bearing wall for the box with a hard metal upper zone, chill sections shaped to form the sides and top of the box, a dry sand core to form the bottom of the box, and means in the flask forming a gate leading upwardly to the space below the core.
11. A mould for a journal box having an integral cylindrical bearing wall, comprising a flask, a chill-section and a sand section united together to form a composite core and arranged with the chill-section on the top and in the mould cavity so as to form the cylindrical bearing wall for the box with a hard metal upper zone, chill sections shaped to form the sides of the box, a chill section shaped to form the top of the box, having a recess to form an equalizer seat of hard metal, and means in the flask forming a gate leading upwardly to the space below the core.
12. A mould for a journal box having an integral cylindrical bearing wall, comprising a flask, a chill-section and a sand section united together to form a composite core and arranged with the chill-section on top and in the mould cavity so as to form the cylindrical bearing wall for the box with a hard metal upper zone, chill-sections to form the sides of the box, a dry-sand core to form the bottom of the box, dry-sand cores to form the ends of the box, and a gate in the bottom-core.
13. A mould for a journal box having an integral cylindrical bearing wall, comprising a flask, a chill-section and a sand section united together to form a composite core and arranged with the chill-section on the top and in the mould cavity so as to form the cylindrical bearing wall for the box with a hard metal upper zone, chill sections to form the sides of the box, a dry-sand core to form the bottom of the box, dry-sand cores to form the ends of the box, a chill-section to form the top of the box, and a gate in the bottom core.
14. A mould for a journal box having an integral cylindrical bearing wall, comprising a flask, a chill-section and a sand section united together to form a composite core and arranged with the chill-section on the top and in the mould cavity so as to form the cylindrical bearing wall for the box with a hard metal upper zone, chill-sections to form the sides of the box, a dry-sand core to form the bottom of the box, dry-sand cores to form the ends of the box, a chill-section to form the top of the box, and a gate in the bottom core.
15. A mould for a journal box having an integral cylindrical bearing wall, comprising a flask, a chill-section and a sand section united together to form a composite core and arranged with the chill-section on top and in the mould cavity so as to form the cylindrical bearing wall for the box with a hard metal upper zone, chill-sections to form the sides of the box, a dry-sand core to form the bottom of the box, dry-sand cores to form the ends of the box, a chill section to form the top of the box, dry-sand cores backing the side top chill sections, and a gate in the bottom core.
16. The combination of claim 14 with a filling of sand under the bottom core and around the side and end cores.
17. The combination of claim 15 with a filling of sand under the bottom core and around the side and end-cores.
- Signed at De Pere, Wisconsin, this 28th day of January, 1929.
- LEE W. MELCHER.